

# United States Patent

[11] 3,622,306

[72] Inventors **Masayuki Tanimura**  
**Yokohama-shi;**  
**Eiichihiro Sunami, Yokohama-shi; Toshio**  
**Nakazawa, Kawasaki-shi, all of Japan**  
[21] Appl. No. **814,276**  
[22] Filed **Apr. 8, 1969**  
[45] Patented **Nov. 23, 1971**  
[73] Assignee **Nippon Kokan Kabushiki Kaisha**  
**Tokyo, Japan**  
[32] Priority **Apr. 8, 1968**  
[33] **Japan**  
[31] **43/22809**

[54] **CORROSION RESISTING LOW ALLOY STEEL**  
**2 Claims, 1 Drawing Fig.**

[52] U.S. Cl. **75/125,**  
**75/126 R**

[50] **Field of Search.....** 75/124,  
**125, 126, Machine Searched**

[56] **References Cited**  
**UNITED STATES PATENTS**  
**2,763,544 9/1956 Wagner .....** 75/125  
**2,845,345 7/1958 Bauscher.....** 75/125

**Primary Examiner—Hyland Bizot**  
**Attorney—Linton & Linton**

**ABSTRACT:** Corrosion resisting low alloy steel having stress-corrosion cracking resistability, good weldability and higher strength under some kind of environment containing  $H_2S$  and the like, which is chiefly composed of Cu-Cr-Al system constituents without addition of strengthening elements such as Ti, Nb, V and the like.





INVENTOR  
MASAYUKI TANIMURA,  
EIICHIRO SUNAMI, AND  
TOSHI NAKAZAWA

BY *Linton and Linton*  
ATTORNEYS

**CORROSION RESISTING LOW ALLOY STEEL**

The present invention relates to economical corrosion resisting low alloy steel having sufficient corrosion resistability and stress-corrosion cracking resistability under some kind of environment containing  $H_2S$  gas and the like.

It is well known that stress-corrosion cracking often occurs in some fields as in the petroleum industry. Accordingly, preventing oil well tubing, valves, bolts, nuts and the like, which are employed in oil fields containing  $H_2S$  gas, from outbreak of the above stress-corrosion cracking, should be further examined. As a matter of fact, reexamination on 9% Ni steel and the like of which the above parts are made is actively done and many studies as to how the composition exerts an influence upon the quality of the parts and upon the occurrences of stress-corrosion cracking has been announced. However, the means of decisively solving said problem are not yet established and are more than deciding the limit of employed stress.

It is an actuality that such a passive means as mentioned above is forced to use. The stress-corrosion cracking in welding place of the above high strength steel is a case in point. Sensibility to the above cracking in welding place is very elevated and is difficult to be relieved, even if a proper heat-treatment is carried out after welding. As mentioned above, the steel keeping resistability for said stress-corrosion cracking, which is owing to sulfide system inclusions in the welding place, is not yet found out.

The features of the present invention are found in Cu-Cr-Al system composition of low alloy steel, which is

pointed out as under-mentioned. Upper limit of C content, i.e. 0.15%, is based on the fact that more than 0.15% C makes corrosion resistability and stress-corrosion cracking resistability worse and also deteriorates its weldability. 0.2% Si and 0.3% Mn is the lower limit content respectively for keeping sufficiently high yield point and tensile strength and more than 0.8% content of Mn deteriorates corrosion resistability or more than 0.6% content of Si increases the brittleness. The reason that P and S is limited to less than 0.03% respectively is 10 on account of accelerating stress-corrosion cracking. Cu is an element of making the corrosion resistability increase and of raising the strength of the steel. However, the above effects in case of less than 0.2% content of Cu are impossible to attain and more than 0.6% content of Cu brings about a difficulty of manufacturing good steel and simultaneously results in injuring stress-corrosion cracking resistability and weldability. Or else shows good stress-corrosion cracking resistability with improved corrosion resistability. If the content of Cr is less than 20 0.2% it is, however, difficult to expect the above effects. More than 1.0% content of Cr has had influence on both workability and weldability of steel. A great quantity of Al, which is possible to make said stress-corrosion cracking resistability of steel improve, results in roughening the skin of ingot and lowering the yield, therefore, Al content is limited to less than 0.2%.

The steel based on the above-mentioned composition is shown in the following table I. In the table, steel A, B, and C stand for the present invention and steel D, E, and F are some kind of ordinary steels.

TABLE I

|                          | C    | Si   | Mn   | P     | S     | Cu   | Cr   | Al    | Y.P. | T.S. | El. |
|--------------------------|------|------|------|-------|-------|------|------|-------|------|------|-----|
| Present invention steel: |      |      |      |       |       |      |      |       |      |      |     |
| A                        | 0.06 | 0.22 | 0.56 | 0.023 | 0.016 | 0.28 | 0.48 | 0.010 | 42.5 | 51.2 | 38  |
| B                        | 0.10 | 0.23 | 0.67 | 0.018 | 0.021 | 0.30 | 0.47 | 0.015 | 33.6 | 50.3 | 38  |
| C                        | 0.13 | 0.34 | 0.55 | 0.022 | 0.022 | 0.35 | 0.43 | 0.190 | 32.3 | 50.6 | 37  |
| Comparative steel:       |      |      |      |       |       |      |      |       |      |      |     |
| D                        | 0.17 | tr   | 0.46 | 0.010 | 0.020 | 0.28 | 0.48 | 0.010 | 20.2 | 41.5 | 47  |
| E                        | 0.14 | 0.25 | 0.62 | 0.078 | 0.024 | 0.30 | 0.47 | 0.015 | 34.6 | 49.0 | 38  |
| F                        | 0.16 | 0.38 | 1.18 | 0.022 | 0.020 | 0.28 | 0.48 | 0.04  | 31.5 | 45.4 | 37  |

chiefly composed of 0.2 to 0.6% Cu, 0.3 to 1.0% Cr and up to 0.20% Al.

An object of the present invention is to provide the steel having corrosion resistability, especially stress-corrosion cracking resistability under a kind of environment containing  $H_2S$  gas and the like.

Another object of the present invention is to provide the steel having a low cost and being able to make the corrosion embrittlement loss reduce by about half in comparison with ordinary high-strength steel.

A further object of the present invention is to provide the steel having higher strength in company with excellent corrosion resistability without special strengthening elements, e.g. Ti, Nb, V and the like.

Additional objects of the present invention will become clear by the following description referring to the examples and the accompanying drawing in which;

The FIGURE is a graph showing stress-corrosion cracking resistability of the present steel in comparison with ordinary corrosion resisting steels.

According to the present invention, the specified chemical composition, by weight percent, is as follows:

|                                              |    |
|----------------------------------------------|----|
| 0.04 to 0.15%                                | C  |
| 0.2 to 1.0%                                  | Si |
| 0.3 to 0.8%                                  | Mn |
| up to 0.03%                                  | P  |
| up to 0.03%                                  | S  |
| 0.2 to 0.6%                                  | Cu |
| 0.3 to 1.0%                                  | Cr |
| up to 0.2%                                   | Al |
| balance being Fe and unavoidable impurities. |    |

In the present invention, the reason for which the chemical composition was determined as mentioned above should be

pointed out as under-mentioned. Upper limit of C content, i.e.

0.15%, is based on the fact that more than 0.15% C makes corrosion resistability and stress-corrosion cracking resistability worse and also deteriorates its weldability. 0.2% Si and 0.3% Mn is the lower limit content respectively for keeping sufficiently high yield point and tensile strength and more than 0.8% content of Mn deteriorates corrosion resistability or

more than 0.6% content of Si increases the brittleness. The reason that P and S is limited to less than 0.03% respectively is 10 on account of accelerating stress-corrosion cracking. Cu is an element of making the corrosion resistability increase and of

raising the strength of the steel. However, the above effects in case of less than 0.2% content of Cu are impossible to attain and more than 0.6% content of Cu brings about a difficulty of

manufacturing good steel and simultaneously results in injuring stress-corrosion cracking resistability and weldability. Or else shows good stress-corrosion cracking resistability with improved corrosion resistability. If the content of Cr is less than

20 0.2% it is, however, difficult to expect the above effects. More than 1.0% content of Cr has had influence on both workability and weldability of steel. A great quantity of Al, which is possible to make said stress-corrosion cracking resistability of steel improve, results in roughening the skin of ingot and lowering the yield, therefore, Al content is limited to less than 0.2%.

The steel based on the above-mentioned composition is shown in the following table I. In the table, steel A, B, and C stand for the present invention and steel D, E, and F are some kind of ordinary steels.

TABLE II

|                             | Test Steel        | Corrosion embrittlement loss mg./cm. <sup>2</sup> |
|-----------------------------|-------------------|---------------------------------------------------|
| 50                          |                   |                                                   |
| The present invention steel | A                 | 7.6                                               |
|                             | B                 | 8.2                                               |
|                             | C                 | 7.8                                               |
|                             | D                 | 15.1                                              |
| 55                          | Comparative steel | 12.9                                              |
|                             | E                 | 19.6                                              |
|                             | F                 |                                                   |

According to the above table II, it is clearly understood that the said corrosion embrittlement loss of this invention steels reduces by half in comparison with the comparative steels. And then, stress-corrosion cracking test is carried out on the above steels. These results are shown in the accompanying FIGURE. Referring now to the FIGURE, the strength of the invention steel, after the above test, has been still kept at the high degree after 200 hours, which is about 40 kg./mm.<sup>2</sup>. On the other hand, the strength of the comparative steel has rapidly lowered to about 20 kg./mm.<sup>2</sup>. It is evident that these results shows excellent properties of this invention steel under some kind of environment containing  $H_2S$  gas and the like.

According to the present invention, it is, moreover, confirmed that proper heat treatment, e.g. quenching and tempering treatment, is possible to be freely carried out on the ground that some strengthening elements such as Ti, Nb, V and the like are not added to the steel.

While this invention has been explained and described with the aid of a particular example thereof, it is to be clearly understood that the invention is not limited thereby.

What is claimed is:

1. Corrosion resisting low alloy steel consisting of the following chemical composition, by weight percent,

|               |    |
|---------------|----|
| 0.04 to 0.15% | C  |
| 0.20 to 0.6%  | Si |
| 0.30 to 0.8%  | Mn |

|             |    |
|-------------|----|
| up to 0.03% | P  |
| up to 0.03% | S  |
| 0.2 to 0.6% | Cu |
| 0.3 to 1.0% | Cr |
| up to 0.20% | Al |

balance being Fe and unavoidable impurities.

2. Corrosion resisting low alloy steel as claimed in claim 1 wherein the content of Al is 0.01 to 0.19%.

\* \* \* \* \*